# EUROPEAN PATENT SPECIFICATION

(11) **EP 0 605 565 B1**
(45) Date of publication and mention of the grant of the patent: **05.06.1996**
(21) Application number: 92920388.3
(22) Date of filing: 16.09.1992
(51) Int. Cl.: D21C 9/153, D21C 11/00

(54) **A METHOD IN OZONE BLEACHING OF PULP**
VERFAHREN ZUM BLEICHEN VON ZELLSTOFF MITTELS OZON
PROCEDE DE BLANCHIMENT DE PATE A L'OZONE

(30) Priority: 17.09.1991 SE 9102693
(43) Date of publication of application: 13.07.1994
(73) Proprietor: Mo och Domsjö Aktiebolag, S-89101 Örnsköldsvik (SE)
(72) Inventor: BRÄNNLAND, Rolf Carl August, S-161 29 Bromma (SE); NOREUS, Sture Erik Olof, S-890 35 Husum (SE)
(74) Representative: Weinhold, Peter, Dr.
(86) International application number: SE9200635
(87) International publication number: WO9306297

(56) References cited:
- DE-A- 2 005 071
- US-A- 4 450 044
- GERALD HOUGH, "Chemical Recovery in the Alkaline Pulping Processes", 1985, Tappi Press, see page 181, line 23 - line 34.

## Description

### Technical field

The present invention relates to a method in bleaching of lignocellulosic material (cellulose pulp) with ozone.

The cellulose pulp can be produced both chemically and chemimechanically. Chemical cellulose pulps are a clearly defined category of cellulose pulps and are comprised, for instance, of sulphite pulp, sulphate pulp and polysulphide pulp. Particularly suitable chemical cellulose pulps are those that have a high viscosity at relatively low Kappa numbers. Belonging to this group of cellulose pulps are sulphate pulps which have been cooked or digested at a high sulphidity, and modified sulphate pulps that have been cooked or digested in accordance with a counterflow method in which white liquor is added also during an advanced stage of the cooking process, and alkaline cellulose pulps which are cooked in the presence of one or more catalysts, for instance in the presence of a quinone compound, such as anthraquinone. Other suitable cellulose pulps are those having the designations MSS-AQ (mini - sulphide sulphite - anthraquinone), Si-Sa-Si (sulphite-sulphate-sulphite) and PS-Si (polysulphide-sulphite), all of which are referred to in the journal "Paperi ja Puu", 5/1989, pp. 509-513.

Particularly suitable chemimechanical pulps are those in which the digestion or cooking process is relatively far reaching and is followed by a mechanical defibering process.

The ozone bleaching process can be applied to unbleached cellulose pulp or cellulose pulp which has been delignified/ bleached in one or more stages.

### Present standpoint of techniques

In recent times, the use of chlorine as a bleaching agent in the delignification of cellulose pulp has decreased drastically for environmental reasons. Instead, chlorine-free bleaching chemicals, such as oxygen and hydrogen peroxide, have been used to bleach cellulose pulp. Ozone bleaching has also become relevant for application on a full scale, i.e. for use in practice. The use of ozone has previously been inhibited among other things because ozone as a bleaching agent has not been sufficiently selective, i.e. the carbohydrates of the cellulose pulp have been seriously damaged from the attack of free radicals, particularly at the large ozone additions (10-15 kg ozone per tonne of pulp), that are often required by such processes. It has been realized that an advantage is afforded in the manufacture of, e.g., chemical cellulose pulp when the pulp is subjected to an extensive, or far reaching, digestion process, i.e. are digested to an extent such that the lignin contents, expressed in Kappa numbers, will be much lower than has earlier been usual and/or to greatly reduce the lignin content of the cellulose pulp in a delignifying stage, for instance an oxygen bleaching stage following the cooking process. Since the cellulose pulp to be ozone bleached has a relatively low lignin content, it is possible to use a comparatively small ozone charge. Furthermore, it has been found possible to control the formation of free radicals by the ozone, by maintaining the ozone treatment process at a low pH, low temperature and a relatively high pulp consistency (for instance, a consistency within the range of 10-35%) and by adding radical capturers.

The desire to maintain a low pH in the ozone bleaching process, i.e. a high degree of acidity, particularly following an alkaline cooking process, will put high demands on the washing equipment for removing of cooking liquor from the cellulose pulp and optionally for removing of oxygen bleaching spent liquor from the cellulose pulp. Despite thorough washing of the cellulose pulp, there is a certain amount of chemically bound alkali in the cellulose pulp and that alkali consumes hydrogen ions when acidifying the cellulose pulp prior to the ozone treatment process. In addition comes the need of acid (hydrogen ions) in order to obtain the hydrogen ion concentration desired when bleaching the cellulose pulp with ozone. Normally, only sulphuric acid is considered for acidification of the cellulose pulp. The use of sulphuric acid for acidification is disclosed in US-A-4,450,044 where a process for bleaching lignocellulosic material with ozone is described wherein the pH value is adjusted to 7 or below using sulphuric acid. The use of, for instance, hydrochloric acid may result in enrichment of chloride in the chemical recovery system, thereby creating corrosion problems.

### Disclosure of the invention

### Technical problem

The waste liquors deriving from the final pulp bleaching stage have hitherto not generally been returned to the chemical recovery system, but they have been discharged to the recipient. The ever increasing demands placed on emissions to the environment have meant that the release of these liquors to the recipient must be reduced to a minimum. This also applies to relatively harmless compounds in the form, for instance, of non chlorinated but oxygen consuming substances.

When substantially all waste liquors from the bleaching process are returned to the chemical recovery system, a number of basic substances, such as sodium and sulphur, become enriched. Some of these substances must then be ejected from the system, either to air or water, in some form. In the worst of cases, this will result in harm to the environment, for instance when sulphur is ejected in the form of sulphur dioxide and/or hydrogen sulphide. The recovery of sodium sulphate from the chemical recovery system is known from G. Hough, "Chemical Recovery in the Alkaline Pulping Processes", Tappi Press, 1985, p. 181. However, for this substance a market cannot be readily found although it is known from DE-A-2 005 071 to prepare sulphuric acid by electrolysis of a sodium sulphate solution.

### Solution

The present invention solves this problem partially and relates to a method in bleaching with ozone lignocellulosic material (cellulose pulp) which has been produced at least partially by chemical processes, in the presence of water and at an acidity, expressed as pH, of 2-5. The method is characterized in that the acidity is sustained during the ozone bleaching process by adding to the system either a sulphuric acid solution or an acid sodium sulphate solution both of which being prepared by electrolysis (or electrodialysis) of an essentially neutral sodium sulphate solution obtained by mixing waste liquor from the ozone bleaching process with waste liquor from an alkaline treatment stage and in that this solution is cooled so as to precipitate sodium sulphate (Na₂SO₄) and in that the sodium sulphate precipitate is removed and dissolved in essentially clean water.

According to the invention, ozone bleaching waste liquor is mixed with waste liquor from-an alkaline treatment stage, for instance in the bleaching department, so as to obtain an essentially neutral solution, which is then cooled so that sodium sulphate (Na₂SO₄) is precipitated, this sodium sulphate precipitate being separated and led away and dissolved in water and the resulting solution is then subjected to an electrolysis or an electrodialysis process.

The remaining mother liquor, which contains essentially organic materials, is transferred to the chemical recovery system. When the sodium sulphate solution contains metals, such as calcium, magnesium or manganese, in harmful quantities, it is appropriate to treat the solution with a hydrogen saturated cation exchanger prior to the electrolysis or electrodialysis stage.

The sodium sulphate solutions obtained, for instance, in the aforedescribed manner, are subjected to electrolysis or electrodialysis in a cell which is provided with anode, cathode and one or more membranes.

The treatment process can be carried out in at least three ways. According to the simplest alternative, the electrolysis is carried out in a cell that is provided with anode, cathode, and a cation selective membrane, wherein sodium sulphate solution is delivered to the anode chamber and water is delivered to the cathode chamber so that an acid solution is formed and oxygen gas is generated at the anode and so that a sodium hydroxide solution is formed and hydrogen gas is generated at the cathode.

According to another alternative embodiment, the electrolysis is carried out in a cell that is provided with anode, cathode an anion selective and a cation selective membrane, wherein sodium sulphate solution is introduced between the two membranes and water is introduced to the anode chamber and the cathode chamber respectively, so that a sulphuric acid solution is formed and oxygen gas generated at the anode and so that a sodium hydroxide solution is formed and hydrogen gas generated at the cathode.

According to a third, more advanced alternative, the treatment is carried out in a multi chamber cell that is provided with anode, cathode and anion selective, cation selective and bipolar membranes, wherein the anode chamber is delimited by an anion selective membrane and the cathode chamber is delimited by a cation selective membrane, and wherein bipolar membranes are disposed between said membranes, and wherein sodium sulphate solution is delivered to those chambers that are delimited by bipolar membranes, so that a sulphuric acid solution is formed in at least the membrane chamber which is placed nearest the cathode and hydrogen gas is generated at said cathode, and so that a sodium hydroxide'solution is formed at least in the membrane chamber which is placed nearest the anode, and oxygen gas is generated at said anode.

According to this third alternative, oxygen gas and hydrogen gas are formed in smaller quantities than in the two preceding alternatives, since these electrode reactions do not take place at the bipolar membranes. This third method is referred to as electrodialysis.

The first and the second alternative methods, i.e. the methods which describe conventional electrolysis, are particularly preferred because of their simplicity.

The acid solution (sulphuric acid solution) and the sodium hydroxide solution respectively formed in the aforesaid cells are removed from the cell individually and the acid solution (the sulphuric acid solution) is delivered to the cellulose pulp so as to obtain the acidity required and desired for the ozone bleaching process. Sodium hydroxide is also a valuable chemical which can be used, for instance, in the alkaline stage of the cellulose pulp treatment process, this stage often following the ozone bleaching stage. If desired, the intrinsically valuable chemicals oxygen and hydrogen can also be collected.

### Advantages

The invention enables the consumption of externally produced (purchased) acid and externally produced (purchased) alkali to be greatly reduced in the manufacture of cellulose pulp that is bleached with ozone. The secondary products oxygen gas and hydrogen gas can be used in the cellulose pulp manufacturing process, for example for oxygen gas bleaching and steam generation respectively. The invention primarily leads to the possibility of mastering the environmental problems in a practically complete closing of the pulp manufacturing process, i.e. also including final bleaching waste liquors. When commercial sulphuric acid is used to achieve the necessary acidity of the cellulose pulp in an ozone bleaching process, it would mean, for instance, that 12,000-18,000 tonnes of sodium sulphate must be ejected per year from the process in an average sized sulphate pulp mill, when this alternative is chosen for maintaining a chemical balance in the system.

### Brief description of the drawings

Figure 1 is a flow sheet which illustrates a pulp manufacturing process in which a first embodiment of the invention is included and described, this embodiment including mixing together ozone bleaching waste liquor and some other alkaline waste liquor.

Figures 2, 3 and 4 illustrate in detail a partial stage of the invention, namely in Figures 2 and 3 the electrolysis of the sodium sulphate solution produced, and in Figure 4, the electrodialysis of the sodium sulphate solution produced.

### Best modes of carrying out the invention

Preferred embodiments of the invention are described in the following with reference to the drawings. An exemplifying embodiment is also described. In connection herewith, the description includes more detailed information as to how the inventive method is carried out.

According to Figure 1 pine chips are delivered through the conduit 1 to the digester 2, which contains a cooking liquor composed essentially of sodium hydroxide and sodium sulphide. Subsequent to digesting the wood and exposing the fibres thereof, the exposed fibres - the pulp - is transported through the pulp conduit 3 (which extends through the entire pulp mill) to the washing section 4, where the major part of the consumed cooking liquor (the cooking waste liquor or the black liquor) is extracted from the pulp. The cooking waste liquor is transported through conduits 5 and 6 to the chemical recovery system of the mill, this system including, among other things, an evaporation plant 7 and a combustion plant (recovery boiler) 8, which is provided with an electric precipitator 9.

Subsequent to washing of the pulp in the washing department 4 and subsequent to optional screening of the pulp (not shown in the drawing), the pulp is passed to an oxygen bleaching stage where the pulp is supplied with oxygen gas, through the conduit 11, and also with alkali, normally sodium hydroxide, and optionally also with a protector. The oxygen bleached pulp is passed to a washing stage 12 in which the pulp is freed from the major part of the waste liquor deriving from the oxygen bleaching stage. The aforesaid treatment process is carried out advantageously in a conventional press or in a washing press to which washing liquid is added. The pulp is brought to the desired consistency for the following ozone bleaching process of the pulp, by adjusting the pressure at which the pulp is pressed. The oxygen bleaching waste liquor pressed from the pulp is passed through the conduits 13 and 6 to the traditional chemical recovery system. Part of the oxygen bleaching waste liquor can be returned to the bottom of the oxygen bleaching reactor 10 through the conduit 14. The pulp, which has a comparatively high pulp consistency is then delivered to the mixer 15 in which an acid sodium sulphate solution is added to the still alkaline pulp, this sodium sulphate solution being prepared in the electrolysis cell 16 and transported through the conduit 17. The acid solution is added in a quantity which will ensure that the pH value of the pulp/water mixture will be suitable for the ozone bleaching of the pulp, i.e. within the range 2-5.

When the pulp leaves the mixer 15, it may, for instance, have a medium pulp consistency (10-15%) or a high pulp consistency (30-35%), depending on requirements. The pulp is then delivered to the ozone bleaching reactor 18 to which oxygen gas containing a given low ozone content is delivered, in addition to pulp, through the conduit 19. The ozone bleaching stage is maintained at a comparatively low temperature, for instance a temperature within the range of 40-60°C. The pulp reacts completely with the ozone in this stage, and residual oxygen gas is led from the reactor through the conduit 20, for transportation to an apparatus for generating fresh ozone (not shown in the Figure). The pulp is then transported to a further washing stage 21, for instance in the form of a washing press. The ozone bleaching waste liquor recovered is passed back to the system, through the conduit 22. The waste liquor is divided into two flows, of which one flow is passed through the conduit 23 back to the ozone bleaching reactor 18 for the purpose of flushing pulp from the reactor. The other flow is passed to a mixing and crystallizing vessel 25, through the conduit 24.

The pulp is then passed to a mixer 26 in which alkali, essentially sodium hydroxide, is added to the pulp. A significant part of the alkali is recovered in the form of a sodium hydroxide solution in the electrolysis cell 16, and the solution is added to the pulp in the mixer 26 through the conduit 27. The remainder of the sodium hydroxide required is supplied externally (purchased alkali) through the conduit 43. The pulp is then passed to an alkalizing or extraction tower 28. In addition to using a plain alkali stage in this stage of the process, it is possible, and even advantageous, to supply also oxygen or peroxide or both of these chemicals. Finally, the pulp is washed in the washing stage 29. It is quite possible to terminate the pulp manufacturing process at this stage and, for instance, to transport the pulp to a paper mill and/or to a dewatering and drying machine for the manufacture of commercial pulp. However, it is often desired to increase both the cleanliness and the brightness of the pulp by undertaking one or more additional bleaching stages while using bleaching chemicals such as, e.g., dithionite, peroxide, chlorine dioxide or additional ozone.

When the bleaching process is terminated at the aforesaid alkali stage, clean water is normally added to the pulp through the conduit 30. The alkaline waste liquor is returned in the system through the conduit 31. The recovered waste liquor is divided into three parts. A first part is added through the conduit 32 to the mixer 26, where it is mixed with the pulp so as to increase its alkali content. A second part is delivered through the conduit 33 to the conduit 24 where the alkaline waste liquor is mixed with the acid ozone bleaching waste liquor so that the waste liquor mixture delivered to the crystallization vessel 25 is generally neutral, i.e. has a pH of 7 or a value in the vicinity thereof. The remaining quantity of waste liquor is passed through the conduit 31 to the pulp washer 4, immediately downstream of the digester 2.

The waste liquor mixture in the vessel 25 is cooled to a temperature of, e.g., 15°C or therebelow. A major part of the sodium sulphate present in the waste liquor will then precipitate in the form of crystals, which settle on the bottom of the vessel 25. The crystals are then passed through the conduit 34 to a washing filter 35, with the aid of an appropriate feeding out device. The waste liquor - mother liquor - freed from the sodium sulphate crystals in the vessel 25 is discharged through the conduit 36 and mixed with oxygen bleaching waste liquor and cooking waste liquor (black liquor) for transportation into the evaporator plant 7.

The sodium sulphate crystals are washed and cleaned on the filter 35 with a small quantity of liquid, and are thereafter passed to the dissolving vessel 38 through the conduit 37. The liquid removed from the sodium sulphate crystals on the filter 35 may, for instance, be introduced in the conduit 36 (not shown in the Figure). Preferably, clean water is passed through the conduit 39 to the dissolving vessel 38 in a quantity such that essentially all sodium sulphate crystals are dissolved. The dissolving process is facilitated by using a temperature which is slightly higher than room temperature and which, for instance, reaches 35°C. The solution containing a large quantity of dissolved sodium sulphate is transported through the conduit 39 to the anode chamber of the electrolysis cell 16. Preferably clean water is delivered to the cathode chamber in the electrolysis cell 16 through the conduit 40. During the process of electrolysis, there is formed at the anode an acid solution which is recovered in the manner earlier described, while at the cathode there is formed a sodium hydroxide solution which is recovered in the aforedescribed manner. Oxygen gas is also generated in the anode chamber, this gas being led away through the conduit 41, while hydrogen gas is generated in the cathode chamber and led away through the conduit 42.

The flow sheet illustrates an application of the invention when bleaching sulphate pulp with ozone, this pulp having been subjected to an oxygen bleaching process prior to the ozone bleaching stage. Reference has earlier been made to suitable final bleaching stage or stages when desiring to further increase the cleanliness and brightness of the pulp. Similarly, it is possible to introduce further delignifying and/or bleaching stages between the digestion stage, i.e. the manufacture of the original pulp, and the ozone bleaching stage. Advantageously, an acid treatment stage can be included, for instance by allowing the pulp to react with a gas that contains nitrogen dioxide (this process is known as PRENOX), immediately prior to the oxygen bleaching stage. In addition to an oxygen bleaching stage in the mentioned position, there can be applied a plain alkali stage, or a peroxide reinforced alkali stage, or an alkali stage which is reinforced with both peroxide and oxygen. Irrespective of whether an acid treatment stage, for instance in accordance with the PRENOX method, is introduced in the mentioned position or not, it may be beneficial to treat (bleach) the pulp with chlorine dioxide, with or without intermediate washing of the pulp, immediately prior to the ozone bleaching stage.

As previously mentioned, the inventive method is in no way limited to the ozone bleaching of sulphate pulp, but can be applied to the ozone bleaching of any chemical pulp whatsoever and also to the ozone bleaching of chemimechanical pulp. When bleaching such pulps, the bleaching sequences can be quite different to the aforedescribed and mentioned bleaching sequences. With regard, for instance, to sulphite pulp, this pulp will have after the digestion stage a much lower lignin content and a much higher brightness than sulphate pulp, which means that only two bleaching stages and at most three bleaching stages, of which one is an ozone bleaching stage, are required in order to obtain a highly clean and bright pulp.

Figure 2 shows in more detail the construction of an electrolysis cell similar to that shown in figure 1 and illustrates how decomposition of the sodium sulphate takes place.

The electrolysis cell 100 is comprised of two chambers, the anode chamber 101 and the cathode chamber 102. An anode 103 is arranged in the first mentioned chamber and a cathode 104 is arranged in the other chamber. The two chambers are mutually separated by a cation selective membrane 105, which will only allow sodium ions to pass through. Sodium sulphate solution is added to the anode chamber 101 through the conduit 106 and water is added to the cathode chamber 102 through the conduit 107. As a result of applying an electric voltage across the cell, hydrogen ions are formed at the anode 103 while generating oxygen gas at the same time, this gas being led away from the cell through the conduit 108. Hydroxide ions are formed at the cathode 104 at the same time as hydrogen gas is generated, this gas being led away from the cell through the conduit 109. The current efficiency in the electrolysis process is greatly dependent on the concentrations of hydrogen ions and hydroxide ions respectively in respective chambers. Consequently, it is not possible in this type of electrolysis cell to produce two hydrogen ions = H⁺, for each sulphate ion = SO$\frac{\text{2-}}{\text{4}}$ and normally it is necessary to be satisfied with a yield of one hydrogen ion or slightly more with each sulphate ion. A part of the sodium sulphate is- therefore still not decomposed. Consequently, the solution removed from the anode chamber 101 through the conduit 110 is designated an acid sodium sulphate solution. A sodium hydroxide solution is removed from the cathode chamber 102 through the conduit 111. The destination of these solutions will be apparent from the earlier description.

When desiring to produce two hydrogen ions for each sulphate ion, i.e. to produce sulphuric acid, an electrolysis cell 120 having three chambers can be used, as shown in Figure 3.

This cell also includes an anode chamber 121 and a cathode chamber 122. An anode 123 is arranged in the anode chamber while a cathode 124 is arranged in the cathode chamber. Located centrally between these two chambers is a further chamber 125 which is encircled by a cation selective membrane 126 which allows sodium ions to pass through, and an anion selective membrane 127 which allows sulphate ions to pass through. Sodium sulphate solution is delivered to the cell through the conduit 128 and is recycled back to the conduit (in a lower concentration) through the conduit 129. Water is delivered to the cell through the conduit 130, to both the cathode chamber 122 and the anode chamber 121.

When an electric voltage is applied over the cell 120, oxygen gas is generated at the anode 123, this gas being led away through the conduit 131, at the same time as sulphuric acid (H₂SO₄ or 2H⁺ + SO$\frac{\text{2-}}{\text{4}}$) is formed in the anode chamber 121. Hydrogen gas is generated at the cathode 124 and is led away from the cell through the conduit 132, at the same time as sodium hydroxide (NaOH or Na⁺ + OH⁻) is formed in the cathode chamber 122. Respective solution is led away from the cell 120 through the conduits 133 and 134 and the chemicals concerned are used in the manner earlier mentioned.

When desiring to reduce the amount of oxygen gas and hydrogen gas formed in relation to the major products acid and alkali in comparison with those electrolysis processes described with reference to Figures 2 and 3, a cell 140 of the type illustrated in Figure 4 can be used.

This cell also has an anode chamber 141 and a cathode chamber 142 having respectively an anode 143 and a cathode 144. The anode chamber 141 is delimited on one side by an anion selective membrane 145, while the cathode chamber 142 is delimited on one side by a cation selective membrane 146. Arranged between these two membranes are two bipolar membranes 147 and between these a further cation selective membrane 146 and an anion selective membrane 145 are arranged. Sodium sulphate solution is added to the anode chamber 141 and the cathode chamber 142 respectively through the conduit 148, and also to each third chamber between the bipolar membranes, which can be included in a greater or smaller number. Water is added to remaining cell chambers through the conduit 149. When an electric voltage is applied across the cell, oxygen gas is generated at the anode 143 and led away through the conduit 150, and hydrogen gas is generated at the cathode 144 and led away through the conduit 151. Furthermore, sodium ions migrate in a direction towards the cathode 144 and sulphate ions migrate in a direction towards the anode 143. The water is dissociated to hydrogen ions and hydroxide ions at the same time. Sulphuric acid (H₂SO₄ or 2H⁺ + SO$\frac{\text{2-}}{\text{4}}$) and sodium hydroxide respectively are formed in this way. Sulphuric acid solution is led away from two of the membrane chambers and transported through the conduit 152 for use in accordance with the earlier description. Sodium hydroxide solution is led away from two other membrane chambers and transported through the conduit 153 for use in accordance with the earlier description. Sodium sulphate solution (of lower concentration) is led away from the bottom of the three chambers where fresh such solution is added to the upper part of the cell and recycled back to the conduit 148, through the conduit 154. The decomposition of sodium sulphate and water illustrated in Figure 4 is normally designated electrodialysis.

It will be understood that other processes of electrolysis respectively electrodialysis can also be applied when carrying out the inventive method.

A number of experiments have been carried out with the method according to the present invention. The manner in which these experiments were carried out and the results obtained will be evident from the following working examples. The experiments concerned were carried out on a pilot-plant scale.

### Example 1

The experiment was carried out with a pine sulphate pulp having a Kappa number of 29.0 and a viscosity of 1,250 dm³/kg. The pulp was oxygen bleached at a pulp consistency of 12% and at an oxygen pressure of 5 kg/cm². 2% sodium hydroxide and 0.3% magnesium in the form of magnesium sulphate (MgSO₄) had earlier been supplied to the pulp. Upon completion of the oxygen bleaching process, the pulp had a Kappa number of 15.0 and a viscosity of 1,010 dm³/kg. The pulp was then pressed to a pulp consistency of 40%. Inorganic chemicals (washing losses) corresponding to 12 kg sodium sulphate per tonne of pulp were found to remain in the pulp. An acid sodium sulphate solution was then added to a pulp flow of 100 kg/min. in an amount of 10 litre/min. The liquid contained 80 g/l of sodium sulphate and hydrogen ions, expressed as sulphuric acid, in an amount of 160 g/l. The pulp concentration fell therewith to 33% and the pH of the pulp-became 2.5.

The pulp was fluffed and introduced into an ozone bleaching reactor, where the pulp was allowed to react with ozone added in a quantity of 0.4 kg/min in a flow of 5.7 kg/min oxygen gas. The temperature was 50°C and the treatment time 30 minutes. The oxygen gas freed from ozone was removed from the reactor. At the end of the treatment time, liquid was added so as to flush away the pulp. Dilution liquid in the form of water was added in an amount of 540 l/min. The pulp was then pressed to a pulp consistency of 30%. The resultant ozone bleaching waste liquor was thereby recovered. The pulp was then transferred to a mixer, to which 2.7 kg of sodium hydroxide/min were added. The pulp was allowed to react with the alkali for 120 minutes at a temperature of 65°C and a pulp concentration of 14%. The pulp was then washed with clean water so as to obtain an alkaline waste liquor.

The Kappa number of the pulp after this treatment stage was 7.3, its viscosity 903 kg/dm³ and its brightness 53% ISO.

The Kappa numbers, viscosities and brightnesses recited in this patent application have been determined in accordance with SCAN-C 1:77, SCAN-CM 15:88 and SCAN-C 11:75 respectively.

The ozone bleaching waste liquor in an amount of 15 l/min., containing 310 g/l sodium sulphate, hydrogen ions, calculated as H₂SO₄, in an amount of 40 g/l and organic material in an amount of 90 g/l, was mixed with the alkaline waste liquor in an amount of 12 l/min so that the resultant pH of the mixture was 7.1. The mixture was transferred to a crystallization vessel, in which the mixture was cooled to 10°C. Sodium sulphate crystals in an amount of 3.3 kg/min were separated from the mixture (the mother liquor) and the sodium sulphate content thereof fell to 90 g/l.

These crystals were then dissolved in a vessel in clean water in a quantity such that the content of dissolved sodium sulphate became 430 g/l. This solution had a temperature of 35°C and was added to the anode chamber of an electrolysis cell of the type illustrated in Figure 3. Clean water was added to the cathode chamber of the cell. The cell temperature was 50°C, the voltage was 3.8 V, the current density was 25 A/dm² and the power consumption was 240 kW.

During the electrolysis process, oxygen gas was generated in the anode chamber in an amount of 190 l/min (0.27 kg/min) at the same time as an acid sodium sulphate solution was formed in which the hydrogen ions, calculated as sulphuric acid, rose to 1.7 kg/min (75% conversion). Hydrogen gas developed in the cathode chamber in an amount of 380 l/min (0.034 kg/min) at the same time as a sodium hydroxide solution was formed in an amount of 14 l/min at a concentration of 10%.

As previously mentioned, the resultant acid sodium sulphate solution contained 80 g/l sodium sulphate and hydrogen ions, expressed as sulphuric acid, in an amount of 160 g/l. The solution concerned was used fully to acidify the pulp prior to the ozone bleaching stage, as earlier described, so that the pulp had a pH of 2.5. The resultant sodium hydroxide solution was added to the pulp, as earlier mentioned, in the mixer prior to the alkalization treatment process. The sodium hydroxide content of this solution covered 50% of the sodium hydroxide addition to the pulp.

The following chemical savings were achieved in this experiment:
Acidifying chemical, calculated as sulphuric acid = 17 kg per tonne of pulp;
Alkalizing chemical, sodium hydroxide = 14 kg per tonne of pulp;
Oxygen gas = 2.7 kg per tonne of pulp.

As earlier mentioned, when practicing the inventive method on a full scale, the oxygen gas can be used in an alklaline treatment stage, for instance in an introductory oxygen bleaching stage.

## Claims

1. A method in bleaching with ozone (18) lignocellulosic material (cellulose pulp) which has been at least partially manufactured chemically (2), in the presence of water at a degree of acidity, expressed as pH, of 2-5,
**characterized in,** that the acidity is maintained during the ozone bleaching process (18) by adding (15) a sulphuric acid solution or an acid sodium sulphate solution (17) both of which being prepared by electrolysis (or electrodialysis) (16) of an essentially neutral sodium sulphate solution (24) obtained by mixing waste liquor (22, 24) from the ozone bleaching process (18) with waste liquor (31, 33) from an alkaline treatment stage (28) and in that this solution is cooled (25) so as to precipitate sodium sulphate (Na₂SO₄) and in that the sodium sulphate precipitate is removed (34) and dissolved (38) in essentially clean water.

2. A method according to claim 1,
**characterized** in that mother liquor obtained from the crystallization of sodium sulphate (25) is transferred (36) to the chemical system which includes the evaporation (7) and combustion plant (8).

3. A method according to Claims 1-2,
**characterized** in that the electrolysis is carried out in a cell (100) which comprises anode (103), cathode (104) and a cation selective membrane (105), wherein sodium sulphate solution is added (106) to the anode chamber (101) and water is added (107) to the cathode chamber (102) so that an acid solution is formed and oxygen gas is generated (108) at the anode (103) and so that a sodium hydroxide solution is formed and hydrogen gas is generated (109) at the cathode (104); and in that respective solution is removed from the cell (110, 111) and in that the acid solution (110) is added to the ozone bleaching process.

4. A method according to Claims 1-2,
**characterized** in that the electrolysis is carried out in a cell (120) which comprises anode (123), cathode (124), and anion selective membrane (127) and a cation selective membrane (126), wherein sodium sulphate solution is added (128) between the two membranes and water is added (130) to the anode chamber (121) and the cathode chamber (122) respectively so that a sulphuric acid solution is formed and oxygen gas is generated (131) at the anode (123) and so that a sodium hydroxide solution is formed and hydrogen gas is generated (132) at the cathode (124); in that respective solution is removed from the cell (133, 134); and in that the sulphuric acid solution (133) is added to the ozone bleaching process.

5. A method according to Claims 1-2,
**characterized** in that the treatment process (the electrodialysis) is carried out in a multi chamber cell (140) which comprises anode (143), cathode (144), anion selective (145), cation selective (146) and bipolar membranes (147), wherein the anode chamber (141) is delimited by an anion selective membrane (145) and the cathode chamber (144) is delimited by a cation selective membrane (146), and wherein the sodium sulphate solution (148) is added to the anode chamber (141) and the cathode chamber (144), and wherein bipolar membranes (147) are disposed between said anion selective membrane (145) and said cation selective membrane (146); and in that water is added (149) to those chambers which are delimited by bipolar membranes (147) so that a sulphuric acid solution is formed at least in the membrane chamber which is situated nearest the cathode (194) and hydrogen gas is generated (151) at said cathode (144), and so that a sodium hydroxide solution is situated nearest the anode (143) and oxygen gas is generated (150) at said anode (143); in that respective solution is removed from the cell (152, 153); and in that the sulphuric acid solution is delivered (152) to the ozone bleaching process.

## Patentansprüche

1. Verfahren zum Bleichen von Lignocellulose-Material (Cellulose-Halbstoff), das zumindest teilweise chemisch (2) hergestellt wurde, mit Ozon in Gegenwart von Wasser mit einem Aciditätsgrad, ausgedrückt als pH, von 2 bis 5, dadurch gekennzeichnet, daß die Acidität während des Ozon-Bleichverfahrens (18) aufrechterhalten wird durch Zugabe (15) einer Schwefelsäurelösung oder einer sauren Natriumsulfatlösung (17), die beide hergestellt wurden durch Elektrolyse (oder Elektrodialyse) (16) aus einer im wesentlichen neutralen Natriumsulfatlösung (24), die erhalten wurde durch Mischen von Abwasserflüssigkeit (22, 24) aus dem Ozon-Bleichverfahren (18) mit Abwasserflüssigkeit (31, 33) aus einer alkalischen Behandlungsstufe (28), und dadurch, daß diese Lösung gekühlt wird (25), um Natriumsulfat (Na₂SO₄) auszufällen, und dadurch, daß der Natriumsulfat-Niederschlag entfernt (34) und in im wesentlichen reinem Wasser gelöst wird.

2. Verfahren gemäß Anspruch 1, dadurch gekennzeichnet, daß die Mutterlauge, die durch die Kristallisation von Natriumsulfat erhalten wurde (25), in das chemische System überführt wird (36), das Verdampfungs- (7) und Verbrennungsanlage (8) einschließt.

3. Verfahren gemäß Anspruch 1 - 2, dadurch gekennzeichnet, daß die Elektrolyse in einer Zelle (100) durchgeführt wird, die eine Anode (103), eine Kathode (104) und eine kationenselektive Membran (105) umfaßt, worin Natriumsulfatlösung der Anodenkammer (101) zugesetzt wird (106) und Wasser der Kathodenkammer (102) zugesetzt wird (107), so daß eine saure Lösung gebildet wird und Sauerstoffgas an der Anode (103) entsteht (108), und so, daß eine Natriumhydroxidlösung gebildet wird und Wasserstoffgas an der Kathode (104) entsteht (109), und dadurch, daß die jeweilige Lösung aus der Zelle entfernt wird (110, 111), und dadurch, daß die Säurelösung (110) dem Ozon-Bleichverfahren zugesetzt wird.

4. Verfahren gemäß Anspruch 1 - 2, dadurch gekennzeichnet, daß die Elektrolyse in einer Zelle (120) durchgeführt wird, die eine Anode (123), eine Kathode (124) und eine anionenselektive Membran (127) und eine kationenselektive Membran (126) umfaßt, worin die Natriumsulfatlösung zwischen den zwei Membranen zugesetzt wird (128) und Wasser der Anodenkammer (121) bzw. der Kathodenkammer (122) zugesetzt wird (130), so daß eine Schwefelsäurelösung gebildet wird und Sauerstoffgas an der Anode (123) gebildet wird (131) und daß eine Natriumhydroxidlösung gebildet wird und Wasserstoffgas an der Kathode (124) entsteht (132), und dadurch, daß die jeweilige Lösung aus der Zelle (133, 134) entfernt wird und daß die Schwefelsäurelösung (133) dem Ozon-Bleichverfahren zugesetzt wird.

5. Verfahren gemäß Anspruch 1 - 2, dadurch gekennzeichnet, daß das Behandlungsverfahren (die Elektrodialyse) in einer Mehrkammerzelle (140) durchgeführt wird, welche eine Anode (143), eine Kathode (144), anionenselektive (145), kationenselektive (146) und bipolare Membranen (147) umfaßt, worin die Anodenkammer (141) von einer anionenselektiven Membran (145) und die Kathodenkammer (144) von einer kationenselektiven Membran (146) begrenzt werden und worin die Natriumsulfatlösung (148) der Anodenkammer (141) und der Kathodenkammer (144) zugesetzt wird und worin bipolare Membranen (147) zwischen der anionenselektiven (145) und der kationenselektiven Membran (146) angeordnet sind, und dadurch, daß Wasser den Kammern zugesetzt wird (149), die von bipolaren Membranen (147) begrenzt werden, so daß eine Schwefelsäurelösung wenigstens in der Membrankammer gebildet wird (194), die der Kathode am nächsten liegt, und Wasserstoffgas an der Kathode (144) gebildet wird (151) und so, daß eine Natriumhydroxidlösung sich der Anode (143) am nächsten befindet und Sauerstoffgas an der Anode (143) gebildet wird (150), und dadurch, daß die jeweilige Lösung aus der Zelle entfernt wird (152, 153) und die Schwefelsäurelösung in das Ozon-Bleichverfahren überführt wird (152).

## Revendications

1. Procédé de blanchiment à l'ozone (18) de matières lignocellulosiques (pâtes de cellulose) qui ont été, au moins partiellement, fabriquées chimiquement (2) en présence d'eau ayant un certain degré d'acidité correspondant à un pH de 2-5, ce procédé étant caractérisé par le fait que l'acidité est maintenue pendant le processus de blanchiment à l'ozone (18) en additionnant (15) une solution d'acide sulfurique ou une solution de sulfate acide de sodium (17), l'une ou l'autre de ces solutions étant préparée par électrolyse (ou électrodialyse) (16) d'une solution de sulfate neutre de sodium (24) obtenue au moyen d'un mélange de lessive épuisée (22, 24), provenant du processus de blanchiment à l'ozone (18), avec de la lessive épuisée provenant d'une phase de traitement alcalin (28), cette solution de sulfate neutre de sodium étant refroidie (25) de manière à précipiter le sulfate de sodium (Na₂SO₄), ce sulfate de sodium précipité étant enlevé (34) et dissous (38) essentiellement dans de l'eau propre.

2. Procédé selon la revendication 1, caractérisé par le fait que la lessive mère obtenue par cristallisation du sulfate de sodium (25) est envoyée au système chimique qui comporte l'installation d'évaporation (7) et de combustion (8).

3. Procédé selon l'une ou l'autre des revendications 1 ou 2, caractérisé par le fait que l'électrolyse est réalisée dans un réservoir (100) qui est pourvu d'une anode (103), d'une cathode (104) et d'une membrane sélectrice des anions (105), réservoir dans lequel la solution de sulfate de sodium est additionnée (106) dans la chambre de l'anode (101) et l'eau est additionnée (107) dans la chambre de la cathode (102), de manière qu'une solution acide soit réalisée et que le gaz oxygène soit produit (108) à l'anode (103), et de manière qu'une solution d'hydroxyde de sodium soit réalisée et que du gaz hydrogène soit produit (109) à la cathode (104), chacune de ces solutions étant enlevée respectivement (110, 111) du réservoir (100) afin que la solution acide (110) soit additionnée dans le processus de blanchiment à l'ozone.

4. Procédé selon l'une ou l'autre des revendications 1 ou 2, caractérisé par le fait que l'électrolyse est réalisée dans un réservoir (120) qui est pourvu d'une anode (123), d'une cathode (124) et d'une membrane sélectrice des anions (127), ainsi que d'une membrane sélectrice des cations (128), réservoir 120 dans lequel la solution de sulfate de sodium est additionnée (128) entre les deux membranes et l'eau est additionnée (130) dans la chambre de l'anode (121) et dans la chambre de la cathode (122) respectivement, de manière qu'une solution acide sulfurique soit réalisée et que du gaz oxygène soit produit (131) à l'anode (123), et de manière qu'une solution d'hydroxyde de sodium soit réalisée et que du gaz hydrogène soit produit (132) à la cathode (124), chacune de ces solutions étant enlevée respectivement (133, 134) du réservoir (120) afin que la solution acide sulfurique (133) soit additionnée dans le processus de blanchiment à l'ozone.

5. Procédé selon l'une ou l'autre des revendications 1 ou 2, caractérisé par le fait que le processus de traitement (l'électrolyse) est exécuté dans un réservoir (140) qui est divisé en plusieurs chambres et qui est pourvu d'une anode (143), d'une cathode (144), de membranes sélectrices des anions (145), de membranes sélectrices des cations (146), ainsi que de membranes bipolaires (147), réservoir dans lequel la chambre de l'anode (141) est délimitée par une membrane sélectrice des anions (145) et la chambre de la cathode (144) est délimitée par une membrane sélectrice des cations (146), et dans lequel la solution de sulfate de sodium (148) est additionnée dans la chambre de l'anode (141) et dans la chambre de la cathode (144), et dans lequel les membranes bipolaires (147) sont disposées entre une membrane sélectrice des anions (145) et une membrane sélectrice des cations (146), de l'eau étant additionnée (149) dans les chambres qui sont délimitées par les membranes bipolaires (147) de manière qu'une solution acide sulfurique soit réalisée au moins dans la chambre à membrane qui est située à proximité de la cathode (144), et que du gaz hydrogène soit produit (151) à cette cathode (144), et de manière qu'une solution d'hydroxyde de sodium soit située à proximité de l'anode (143) et que du gaz oxygène soit produit (150) à cette anode (143), chacune de ces solutions étant enlevée respectivement (152, 153) du réservoir (140) afin que la solution acide sulfurique soit fournie (152) au processus de blanchiment à l'ozone.
